

## UNITED STATES PATENT OFFICE

WILLIAM F. RICHTER, OF APOLLO, PENNSYLVANIA, ASSIGNOR TO CHEMICAL HOLDING CORPORATION, OF APOLLO, PENNSYLVANIA, A CORPORATION OF DELAWARE

## FABRICATION OF VISCOSE

No Drawing.

Application filed October 7, 1930. Serial No. 487,026.

This invention relates to the fabrication of viscose into useful products, especially to the production of artificial silk. The precipitating baths used commonly at the present time for viscose contain relatively large amounts of sulfuric acid, for example 8 per cent or more, together with rather high concentrations of one or more salts, such as sodium or magnesium sulfates. Such baths, which characterize commercial practice prior to my invention, are open to certain objections. For example, as a result of the rather high concentrations of salts used, the yarn leaving the bath carries away relatively large amounts of salts, so that the baths become depleted quickly, which necessitates renewal of their salt components. Furthermore, the salts usually used tend to crystallize readily, and thus the yarn may become encrusted with them prior to washing. In consequence, not only must the yarn be subjected to prolonged washing, but also the removal of the crystallized material from its fibers may weaken the resultant product.

The objects of this invention are to provide an improved process of precipitating viscose, in which use is made of baths having not only a lower concentration of acid than those used heretofore, but also of salts, and having substituted for the salts now used others better suited for this purpose, whereby crystallization of salts upon the yarn is minimized and there is less danger of weakening of the thread during and after precipitation, and less frequent renewal of salts is necessary.

I have found, and it is upon this that the invention is predicated, that particularly favorable results are obtained in the fabrication of viscose through the use of a precipitating or spinning bath containing sulfuric acid, bismuth sulfate, and zinc sulfate. The invention is applicable to the fabrication of viscose into the various products which are made therefrom, all such products being defined herein as artificial fibers. In the use of baths containing sulfates of bismuth and zinc, lower concentrations of acid may be used than have heretofore been applied commercially, the exact concentration depending upon the product desired. In general it is

preferred to have the bismuth sulfate present in an amount in excess of the zinc sulfate.

The invention is especially applicable to the production of artificial silk. In this embodiment the bath most suitably contains from about 5 to 7 per cent of sulfuric acid, from about 1 to 3 per cent of bismuth sulfate, and from about 0.5 to 2 per cent of zinc sulfate. The proportions here given refer to the anhydrous salts. My tests have shown that particularly suitable results are obtained with a bath of the following composition:

|                 |    |
|-----------------|----|
| Sulfuric acid   | 6% |
| Bismuth sulfate | 2% |
| Zinc sulfate    | 1% |

The bath is preferably used at an elevated temperature, for example between 35° to 50° C., and most suitably between 40° and 45° C. As thus used, the practice of the invention provides lustrous silk of high quality.

Through the use of these bismuth sulfate-zinc sulfate baths the salts are not removed as rapidly by the yarn as has been the case with prior baths, and therefore less frequent renewal of the salts, or replacement of the baths, is necessary. Furthermore, the salts used in the practice of the invention do not possess the strong tendency toward crystallization that is possessed by sodium and magnesium sulfates, and the others which have been commonly used, so that there is less tendency for them to crystallize in the yarn. Because of this, and because the yarn carries out so small an amount of salts, weakening of the yarn through crystallization and washing out of salts is minimized or eliminated. Other advantages, such as reduction in the amount of wash water needed, also attend the invention.

According to the provisions of the patent statutes, I have explained the principle and mode of operation of my invention, and have illustrated and described what I now consider to represent its best embodiment. However, I desire to have it understood that, within the scope of the appended claims the invention may be practiced otherwise than as specifically illustrated and described.

I claim:

1. In a process of preparing artificial fibers from viscose the step comprising precipitating the viscose in a bath containing from about 5 to 7 per cent of sulfuric acid, about 1 to 3 per cent of bismuth sulfate, and about 0.5 to 2.0 per cent of zinc sulfate.
2. In a process of producing artificial silk from viscose the step comprising precipitating the viscose in a bath containing from about 5 to 7 per cent of sulfuric acid, bismuth sulfate, and zinc sulfate in an amount less than said bismuth sulfate.
3. In a process of preparing artificial fibers from viscose the step comprising precipitating the viscose in a bath containing sulfuric acid in an amount sufficient to coagulate the viscose but not exceeding about 8 per cent, and also containing bismuth sulfate and zinc sulfate.

In testimony whereof, I sign my name.

WILLIAM F. RICHTER.

25

30

35

40

45

50

55

60

65